

UNITED STATES PATENT OFFICE

IRVING F. LAUCKS AND GLENN DAVIDSON, OF SEATTLE, WASHINGTON, ASSIGNEES TO  
I. F. LAUCKS, INCORPORATED, OF SEATTLE, WASHINGTON, A CORPORATION OF  
WASHINGTON

VEGETABLE GLUE AND METHOD OF MAKING SAME

No Drawing. Original application filed October 29, 1923, Serial No. 671,381. Divided and this application filed October 4, 1928. Serial No. 310,425.

The art of making a water-proof glue from certain protein materials has been known for some time; thus casein and blood albumin are in common use. These last mentioned compounds, however, have a number of disadvantages from a practical standpoint. Casein is costly and lack of uniformity in the material as derived from various sources is a serious detriment; while blood albumin is not available except in certain situations. There is accordingly a great demand for a new glue that will be cheap and at the same time sufficiently waterproof.

By waterproof, in this connection, it is not meant that glues thus characterized will resist the action of water indefinitely, but it is meant that they are waterproof in the sense in which the term is used in the industry.

Vegetable compounds have not, so far as we are aware, been heretofore satisfactorily employed as a basis for waterproof glues of the type in question. It is true that some veneer makers, on account of the high price of casein have come to use starch glues, but these, at least as heretofore made, are not at all waterproof.

We have now discovered however that by subjecting the material to proper treatment, vegetable matter containing proteins, and starch, can be converted into a waterproof glue that will satisfy certain requirements. The requisite raw material may be derived from a number of sources and the treatment of such material is relatively simple and inexpensive so that as a result we are able to produce a satisfactory glue at a much lower cost than has heretofore been possible.

To the accomplishment of the foregoing and related ends, the invention, then, consists of the combination of ingredients or composition of matter and the steps involved in the preparation of such composition hereinafter fully described and particularly pointed out in the claims, it being understood that such disclosed ingredients and steps constitute but several of the various ways in which the principle of the invention may be used.

Where soya bean flour is employed as raw material, such flour is preferably made by

grinding the soya bean cake so that 80 per cent. will pass a 100 mesh screen, and when treated with certain chemicals, or other substances, we make therefrom a very satisfactory glue. Such bean cake as analyzed by us, is found to contain on the average 45 per cent. protein, 12 per cent. water, 5 per cent. cellulose or crude fiber, 7 per cent. oil, 6 per cent. ash, and 25 per cent. carbohydrates.

We do not, however, wish to limit ourselves to soya bean flour or to vegetable protein derived from this source for we have made satisfactory glue by our improved process from a low grade wheat containing approximately 10 per cent. protein, and there are many other vegetable materials that may be utilized.

Where soya bean flour is employed, it is preferably made from cake from which the oil has been expressed, because it is cheaper and makes a better glue, but flour made from the whole beans, without expressing the contained oil, may also be used, although obviously this would not be economical in view of the value which attaches to such oil. As to the fineness of the flour, it is not necessary that the meal be ground as fine as indicated above, but fineness is desirable from a practical standpoint.

The use of caustic soda with such vegetable matter is desirable, such caustic soda apparently playing the part of dispersing the colloidal material.

As equivalents of such caustic soda, caustic potash and ammonia may be used, although more expensive. Other equivalents of caustic soda in the presence of lime are salts of soda (or potash) with weak acids, e. g. sodium phosphate, sodium borate and the like.

In order to improve the working properties, and the water resisting properties, we add substances of which the following are examples:

Portland cement or other hydraulic cements.

Rosin, sodium or calcium soaps of rosin.

We have also found that certain substances will act in the same way as the caustic soda and also as thinners, e. g. sodium phosphate, sodium perborate and sodium sulphite. These

salts are all related in that they are combinations of the strong base sodium with a weak acid and there are a number of other salts that fall in the same category and which have a similar effect, so need not be listed in detail.

As examples we may cite the following:—

(1) Mix 30 parts low grade wheat flour, 10 parts Portland cement, 30 parts water, 10 parts 18 per cent. caustic soda solution, warm to 80° cent.; add 15 parts water glass.

(2) Mix 30 parts low grade wheat flour, 2 parts sodium dichromate, 5 parts Portland cement, 70 parts water, 20 parts 18 per cent. caustic soda solution.

(3) Mix dry, 40 parts soya bean flour, 6 parts rosin, 8 parts Portland cement, 3 parts dichromate of soda, and 5 parts caustic soda; add 140 parts water and 14 parts water glass; 20 stir well; add 50 parts water.

The particular order in which the several ingredients are admixed together in the formulæ just given may be varied, and it is unnecessary that the manufacture of the product be completed in a single continuous operation, but as a matter of practice, we have found it desirable in certain cases to mix only certain of the ingredients initially and then add the others just before the glue is required for use. Thus the vegetable seed flour, rosin and Portland cement may be mixed dry, and in this form be shipped. Such dry product is then mixed with water, caustic soda solution and sodium silicate in the form of water glass, thereby making a finished glue.

It will also be understood of course, that the foregoing formulæ are typical and that many variations are actually made therein in the compounding of our improved glue.

The formulæ, wherein low grade wheat flour is used, have under test resisted the action of water for thirty-six hours.

We have found that even where the vegetable material contains practically no protein but only starch as a glue making constituent, by using Portland cement, starch being substituted in formula No. 1 for the low grade wheat flour, a glue is obtained much superior to any starch glue at present on the market.

This application is a division of our application Serial No. 671,381, filed October 29, 1923. (Patent No. 1,689,732).

Other modes of applying the principle of our invention may be employed instead of the one explained, change being made as regards the process herein disclosed or the materials employed in carrying out such process provided the stated ingredients and steps or the equivalent of such stated ingredients or steps be employed.

We therefore particularly point out and distinctly claim as our invention:—

1. A glue composition, comprising wheat flour, an alkaline medium, and Portland cement, the proportions of the flour and the

Portland cement being about 30 parts of the former and about 5-10 parts of the latter.

2. The method of making a glue, which comprises treating a vegetable material containing starch with an alkaline medium and a hydraulic cement.

3. The method of making a glue, which comprises treating a vegetable material containing protein and starch with an alkaline medium and a hydraulic cement.

4. The method of making a glue, which comprises treating wheat flour with an alkaline medium, and Portland cement.

5. The method of making a glue, which comprises treating wheat flour with an alkaline medium and Portland cement, in the proportions of about 30 parts of the flour and about 5-10 parts of the Portland cement.

6. A glue composition, comprising the reaction products of vegetable material containing starch, an alkaline medium and a hydraulic cement, in the presence of water.

7. A glue composition, comprising the reaction products of vegetable material containing protein and starch, an alkaline medium and a hydraulic cement, in the presence of water.

8. A glue composition, comprising wheat flour, an alkaline medium and Portland cement, in the presence of water.

9. A glue composition, comprising the reaction products of vegetable material containing starch, caustic soda, and a hydraulic cement, in the presence of water.

10. A glue composition, comprising the reaction products of vegetable material, containing protein and starch, caustic soda, and a hydraulic cement, in the presence of water.

IRVING F. LAUCKS.  
GLENN DAVIDSON.

100  
105

110

115

120

125

130